

# UNITED STATES PATENT OFFICE.

WINFIELD S. POTTER, OF NEW YORK, N. Y.

## MANUFACTURE OF MANGANESE STEEL.

968,601.

Specification of Letters Patent. Patented Aug. 30, 1910.

No Drawing.

Application filed May 20, 1910. Serial No. 562,874.

*To all whom it may concern:*

Be it known that I, WINFIELD S. POTTER, a citizen of the United States, and whose post-office address is 30 Church street, borough of Manhattan, city of New York, county of New York, and State of New York, have invented certain new and useful Improvements in the Manufacture of Manganese Steel; and I do hereby declare the following to be a full, clear, and exact description of the invention, such as will enable others skilled in the art to which it appertains to make and use the same.

My invention relates to the preparation of manganese steel in such form and with such physical characteristics as will permit it to be rolled, forged, or otherwise shaped to advantage. To this end, I produce, in accordance with my invention, a manganese steel ingot, devoid of dendrites and other objectionable freezing structures and of a strong uniform fine grained structure throughout, by means of a series of steps which are closely related to each other and which co-act to bring about with certainty the desired result. This series of steps begins with the treatment of the molten metal itself before the ingots are cast, and continues with the subsequent reconstruction of the ingot desirable for adapting it to successful commercial rolling, forging or shaping.

My invention is based upon the discovery that, by suitably deoxidizing and cleansing the molten metal, as hereinafter described, while still in the furnace, casting ladle or like source of supply, it is possible to standardize the subsequent heat treatment of the cast ingot, and, particularly, for steel of any given composition, to practically eliminate variations in that part of the heat treatment of the ingot which determines the reconstruction of the dendritic portion and its conversion into the strong uniform fine grained structure desired.

The invention is further based upon the discovery that the preliminary deoxidation and cleansing of the metal has the function of establishing a practically definite and short period of time for the complete conversion of the dendrites, thereby enabling the operator to promptly terminate that stage of the heat treatment, which would otherwise tend to the formation and building up of large and coarse crystals, or grains.

In order to further illustrate and make clear the generic character of the invention and the principles of operation upon which it is based, I will now describe a suitable specific method or series of operations for putting it into practice so as to realize its characteristic advantages, and, for this purpose will assume that in the particular instance given, the manganese steel is to be compounded from suitably dephosphorized and desulfurized molten open hearth steel from an open hearth furnace, and molten ferro-manganese, mixed in the desired proportions in a casting ladle of large capacity or other suitable container appropriate for the purpose. However, as hereinbefore indicated, the operations of compounding the metal, deoxidizing and cleansing it, may be effected in the open hearth or other like furnace itself, although, in the case of this very readily oxidized metal, the most complete deoxidizing, cleansing and washing can only be secured by continuing those operations in the ladle itself and with the employment of the protective cover of acid slag as herein-after described.

Assuming that the compounding of the metal is to be effected in the casting ladle of large capacity, (say sixty tons or more) the ladle will be lined with the usual silicious or acid lining, preheated in the customary manner. The charge of dephosphorized molten steel from the open hearth or like furnace will then be run into the ladle and simultaneously therewith the molten ferro-manganese will likewise be charged therein. As the charge of molten metal rises in the ladle, it is essential for the purpose of my present invention to maintain upon its upper surface a protecting layer of acid slag. For this purpose, the ladle may, if desired, be charged with a small quantity of readily fusible acid slag making materials, or a mixture which will form a readily fusible acid slag, before the steel is running from the furnace; or in lieu thereof, or in addition thereto, the acid slag making material may be added from time to time to the charge, as the level of the metal rises in the ladle. The acid slag making materials may conveniently consist of silica or other silicious material associated with a sufficient amount of fluxing ingredients such as sodium silicate, lime, or lead oxid, to make it readily fusible at a sufficiently low temperature, and the proportion of silica should be

sufficient to balance the oxids present in the steel, (as, for instance, the oxid of iron and oxid of manganese) which it is the purpose of my invention to eliminate, as far as possible, by the treatment proposed. The purpose of charging the acid slag making materials into the ladle either before or during the charging of the molten steel is, furthermore, to obtain such an intimate contact of the acid slag formed and the metal as to insure, to the greatest extent possible, the washing out of the oxids from the steel throughout the entire mass thereof. Usually, it will not be found feasible to charge the steel from the open hearth or other furnace into the ladle without likewise encumbering it with a practically unavoidable proportion of the furnace slag containing basic oxids; and, it will be understood that the amount of acid slag making materials to be charged into the ladle should be sufficient to likewise balance and neutralize these basic oxids from the furnace. In fact, the quantity of acid slag making materials charged into the ladle should be somewhat in excess of that required both for cleansing the steel from its contained oxids and also for balancing the oxids admitted from the furnace with the furnace slag, in order that the body of slag finally floating upon the charged metal in the ladle shall be devoid of any oxidizing effect upon the charge. In charging the molten steel into the ladle it will, of course, be understood that it is preferable to avoid as far as possible the entrance of any large portion of the furnace slag. This may be effected in any suitable manner, as, for instance, by diverting the slag over the side of the furnace spout into a slag receptacle.

Tilting furnaces may be used to advantage for the production of the steel, and the opening through which the metal is discharged from the furnace will be made of such size and the furnace so tilted during the pouring operation that the steel enters the ladle with but little slag, whereupon the slag may be afterward poured separately into another receptacle. After the ladle is filled, the metal with its protecting top layer of acid slag is permitted to remain at rest for a period sufficient to insure the separation of the slag and metal, and is permitted to cool to the temperature desirable for casting or teeming into the ingot molds.

In order to effect an entirely satisfactory cleansing of the metal in the ladle, it should be at a relatively high temperature during the cleansing operation, as compared with the temperature of final pouring into the ingot molds. For instance, the cleansing operation may be carried on with the metal at a temperature of say 1400° C. to 1450° C. The metal in the ladle will preferably contain about 12% of manganese and from 80% to 1.10% of carbon; and, in order to

have as little piping as possible in the ingots and to permit the metal to set without undue delay in the molds, the metal in the ladle should be cooled, or permitted to cool, before the pouring operation begins, to a temperature of say 1375° C. The pouring from the ladle is effected through a bottom pouring aperture, and the temperature of the metal and the attendant conditions are to be so established that the metal will set in the ingot molds promptly, with the exception, perhaps, of a small proportion in the innermost longitudinal center or core of the ingot. While the ingot is still in the mold, I preferably cool it in such manner that, when stripped from the mold, the outer portions (to a depth fully including the thickness of the zone of the dendrites) will have an average temperature in the neighborhood of 1000° C., (say from 950° C. to 1050° C.) except at the edges where it will be unavoidably considerably lower. This enables it to be transferred, without suffering any rupture, into a soaking pit or other like heating furnace, wherein it is to be subjected to the heat treatment designed for reconstructing its exterior portions; and it also permits this heat treatment to take place without cracking the ingot. At the time of its entrance into the soaking pit or like furnace, the ingot has set and developed its freezing structures to a depth of say six inches or more inwardly from its outer skin or periphery and a zone of dendrites has formed which usually occupies say about one-half of this depth. In order to break down these dendrites and to substitute therefor a strong uniform structure of fine grain, I then slowly raise the temperature of the soaking pit to 1175° C. or a somewhat higher temperature slowly or evenly, this rise in temperature being effected in a smoky or reducing atmosphere, so that the periphery of the ingot will not be oxidized. I have found that with the preliminary deoxidation and cleansing of the metal, as hereinbefore described, the breaking down of the dendrites and the substitution therefor of a strong uniform fine grained structure can be accomplished at or about the temperature of 1175° C. specified, within a comparatively short period of time, say half an hour, the temperature and the time of reconstruction varying somewhat with the particular composition of the metal, but within relatively narrow limits, one way or the other, from the temperature and the period of half an hour referred to. I have also found that, for steel of any given composition or analysis, the preliminary deoxidizing and cleansing step permits the operator to predetermine the temperature and the time necessary for the desired breaking down of the dendrites and the reconstruction of the steel. So that, not only is the period referred to shortened, but the operation as a

whole is so standardized that the desired result can be anticipated with confidence. After the ingot has remained at the temperature of 1175° C. or thereabout for the period necessary for the reconstruction desired, this stage of the heat treatment is arrested by lowering the temperature so as to prevent the building up within the mass of larger and coarser grains. To this end, the temperature prevailing within the soaking pit or other heating furnace may be lowered by the injection of water vapor, in the form of a steam jet, carrying with it water in suspension, with the result that the periphery of the ingot is reduced in temperature to say 1100° C.; or for the same purpose, the ingot may be cooled by transferring it into a cooler soaking pit, for example. The lowering of the temperature of the exterior portions of the ingot is accompanied with the formation of a tough thick skin, which shrinks upon and works the still plastic interior. Finally, after the cooling of the outer portions of the ingot has occurred, and the steam jet has been cut off, the outer portions of the ingot are preferably permitted to rise again in temperature to say 1125° C., in order to equalize the surface temperatures and to obtain the desirable maximum ductility, whereupon the ingot may be removed from the soaking pit and is in condition to be immediately rolled into rails or other products, in mills of ordinary construction. Moreover, the temperature conditions are such that a track rail, for instance, of standard length and section, rolled from such an ingot, will be delivered from the final pass of the rolls at a temperature which will permit it to be toughened by quenching without being first subjected to a reheating operation.

It will be understood that the cooling temperature of 1100° C. and the reheating temperature of 1125° C. referred to are not to be regarded as absolute. They are the temperatures which are appropriate to manganese steel of what may be termed a soft analysis, that is, having, say, 1.10% of carbon, or less, whereas, when the percentage of carbon is higher, say, 1.20%, and upward, the temperature of cooling will be somewhat lower, and the temperature to which the steel may be reheated will also be lower. In other words, these temperatures will depend upon the analysis of the steel, especially with regard to its content of carbon.

As hereinbefore stated, the preliminary step of deoxidizing and cleansing the manganese steel has for its effect not only to permit the shortening and standardizing of the period in which the dendrites are broken down and converted into a uniform fine grained structure, but by clearing the metal of its oxids throughout, makes it correspondingly stronger as a final product and less tender during the manipulation to

which it is subjected from the time the ingot is cast until the rolling operation is completed. Furthermore, the preliminary deoxidation and cleansing of the metal will permit, to great advantage, the practice of an alternative way of toughening the outer portions of the ingot instead of subjecting it to cooling in the soaking pit. That is, the ingot may be taken from the soaking pit, in which it has been slowly and evenly heated to a temperature of from 1175° C. to 1225° C., depending upon the analysis of the metal, and is then subjected to light mechanical working over its periphery for the purpose of producing a wrought thick skin thereon. The lower temperature (1175° C., or thereabout) is preferred when the amount of carbon present in the ingot is above 1.20%; and the higher temperature (1225° C., or thereabout) is preferred when the amount of carbon present is 1.10%, or less, it being assumed in both of these instances that any phosphorus present is low in amount. The preliminary deoxidizing and cleansing operation greatly facilitates the welding of this outer skin and also makes it possible to execute this step of the operation at a higher temperature. This welding or consolidating of the outer portions of the ingot to produce a wrought skin or shell is of particular importance where the reduction contemplated in the rolling mill is considerable for the initial passes thereof. It is carried out quickly, so that there may be no material drop in temperature, and the ingot is then delivered to the rolling mill and rapidly reduced in the usual manner.

In order to give a concrete instance of the light preliminary working appropriate to the practice of the invention, I will assume that the manganese steel ingot is a 20x20" square section. The light preliminary rolling would be effected by acting first simultaneously upon two horizontal sides, and then turning the ingot and acting simultaneously upon the two remaining sides. Where the analysis of the manganese steel of the ingot shows it to be low in carbon (say containing 1.10% of carbon, or somewhat less than that amount), the reduction in the first one or two passes of the preliminary light rolling may be about one inch in each pass. This first reduction along the two horizontal sides of the ingot renders the metal of those sides capable of greater elongation, and consequently, when the ingot is turned over and rolled along its opposite sides, a somewhat greater reduction can take place, say one and one-half or one and three-quarter inches. These two preliminary reducing passes will in general suffice for the light preliminary rolling intended, although, in some instances, they may be supplemented by a third or even a fourth pass, if the mill conditions

are such that the light preliminary rolling can be effected quickly. When the manganese steel has a harder analysis, *i. e.*, when the percentage of carbon is as high as 1.20%, 5 or higher, it will usually be advisable to limit the first reductions of the series of light preliminary passes to from one-half to three-quarters of an inch, it being permissible, however, to somewhat increase the reduction in the subsequent pass or passes, for 10 the reason hereinbefore explained, *i. e.*, because the metal of those sides which have been subjected to the action of the reducing rolls is capable of greater elongation for the 15 next succeeding pass.

When an electric furnace is used for the making or compounding of the manganese steel, and when there is present in that furnace a considerable proportion of manganese, it is difficult to avoid the production 20 of a large amount of manganese oxid. To meet this difficulty, it will be desirable, just before the metal is tapped from the electric furnace into the ladle, to add to the furnace 25 charge a reducing agent (such as silico-calcium, aluminum, ferro-titanium, or the like) in sufficient quantity to properly reduce the oxid contained in the metal. The metal would then be charged into the ladle, as free 30 as possible from the furnace slag. In view of the highly oxidizable character of the metal, further oxidation will take place during the transfer of the metal from the furnace into the ladle, and therefore the final 35 deoxidation, cleansing and washing of the steel will proceed in the ladle as hereinbefore described.

As has been hereinbefore indicated, the temperature of the ingot may be raised in 40 the soaking pit, in some instances, to a degree higher than 1175° C. in its exterior portions; in fact, to somewhat exceed this limit, (say by bringing the temperature of the exterior portions to 1225° C.) will be 45 found useful in most instances in order to insure greater reliability in case the casting conditions should be more or less unfavorable to the operation, and in order to obtain a correspondingly greater ductility of 50 the metal during its passage through the rolls.

What I claim is:

1. In the production of manganese steel ingots, the step of preliminarily cleansing the 55 manganese steel, while in the molten condition and before casting into the ingot mold, by converting the oxid contained therein into more readily separable compounds and permitting said compounds to separate out 60 by flotation, and preserving the molten metal from surface oxidation thereafter by maintaining thereon a protective layer of non-basic slag; substantially as described.

2. In the production of manganese steel 65 ingots, the step of preliminarily cleansing the

manganese steel, while in the molten condition and before casting into the ingot mold, by converting a portion of the oxid contained therein into more readily separable compounds and permitting said compounds 70 to separate out by flotation, and reducing other portions of said oxid by the introduction into the molten metal of a reducing agent; substantially as described.

3. In the production of manganese steel 75 ingots, the step of preliminarily cleansing the manganese steel, while in the molten condition and before casting into the ingot mold, by intimately mixing and washing the steel with silica, thereby separating out 80 contained oxid as silicates, and separating the silicates by flotation, and thereafter maintaining a protecting layer of the acid slag upon the top of the metal; substantially as described.

4. In the production of manganese steel 85 ingots, the step of obtaining the metal in suitable condition for making the desired ingot, by mixing in an acid-lined ladle a body of molten steel from a furnace and a 90 body of molten ferro-manganese, diverting the major portion of the furnace slag so that it will not enter the ladle, and neutralizing or balancing such portion of the furnace slag as may enter the ladle by introducing into the ladle a sufficient amount of acid material for that purpose; substantially 95 as described.

5. In the production of manganese steel 100 ingots and their subsequent heat treatment in order to remove their objectionable freezing structures, the preliminary step of cleansing and deoxidizing the metal from which the ingot is cast, to an extent sufficient to substantially eliminate the variations in the temperature necessary for the reconstruction desired, and subjecting the ingot to the reconstructing temperature until the objectionable freezing structures have 105 been removed; substantially as described.

6. In the production of manganese steel 110 ingots and their subsequent heat treatment in order to convert their dendrites into structures of uniform fine grain, the preliminary 115 step of cleansing and deoxidizing the metal from which the ingot is cast to an extent sufficient to substantially eliminate variations in the temperature necessary for the reconstruction desired, and subjecting the ingot to the reconstructing temperature until the desired uniform fine crystalline structure has been produced; substantially as described.

7. In the production of manganese steel 120 ingots and their subsequent heat treatment in order to convert their dendrites into structures of uniform fine grain, the preliminary 125 step of cleansing and deoxidizing the metal from which the ingot is cast to an extent sufficient to substantially eliminate va- 130

riations in the temperature necessary for the reconstruction desired, cooling the ingot until the exterior portions have temperatures in the neighborhood of 1000° C., and subjecting the ingot to the reconstructing temperature until the desired uniform fine crystalline structure has been produced; substantially as described.

8. In the production of manganese steel ingots and their subsequent heat treatment in order to convert their dendrites into structures of uniform fine grain, the preliminary step of cleansing and deoxidizing the metal from which the ingot is cast to an extent sufficient to substantially eliminate variations in the temperature necessary for the reconstruction desired, and subjecting the ingot to the reconstructing temperature until the desired uniform fine crystalline structure has been produced, and lightly working the ingot so as to produce a tough wrought skin; substantially as described.

9. In the production of manganese steel ingots and their subsequent heat treatment in order to convert their dendrites into structures of uniform fine grain, the preliminary step of cleansing and deoxidizing the manganese steel containing about 12% Mn. and about 1.10% C. from which the ingot is cast to an extent sufficient to substantially eliminate variations in the temperature necessary for the reconstruction desired, subjecting the ingot to the reconstructing temperature until the desired uniform fine crystalline structure has been produced, and lightly working the ingot so as to produce a tough wrought skin; substantially as described.

10. In the production of manganese steel ingots and their subsequent heat treatment in order to remove their objectionable freezing structures, the preliminary step of cleansing and deoxidizing the metal from

which the ingot is cast to an extent sufficient to substantially eliminate variations in the temperature necessary for the reconstruction desired, casting the metal at a temperature but slightly above its freezing or setting point, cooling the outer portions of the ingot to about 1000° C., and subjecting the ingot to the reconstructing temperature until the desired fine crystalline structure has been produced; substantially as described.

11. In the production of manganese steel ingots and their subsequent heat treatment in order to remove their objectionable freezing structures, the preliminary step of cleansing and deoxidizing the metal from which the ingot is cast to an extent sufficient to substantially eliminate variations in the temperature necessary for the reconstruction desired, casting the metal at a temperature approximating 1375° C., and heating the ingot slowly and evenly to from 1175° C. to 1225° C.; substantially as described.

12. In the production of manganese steel ingots and their subsequent heat treatment in order to remove their objectionable freezing structures, the preliminary step of cleansing and deoxidizing metal from which the ingot is cast to an extent sufficient to substantially eliminate variations in the temperature necessary for the reconstruction desired, casting the ingot at a temperature approximating 1375° C., cooling it to a temperature of about 1000° C., and slowly and evenly heating it to from 1175° C. to 1225° C.; substantially as described.

In testimony whereof I affix my signature, in presence of two witnesses.

WINFIELD S. POTTER.

Witnesses:

JOHN C. PENNIE,  
WILLIAM H. DAVIS.